

Patented Aug. 31, 1926.

1,597,717

# UNITED STATES PATENT OFFICE.

HUBERT BRÄUNLICH, OF FREIWALDAU, CZECHOSLOVAKIA.

## PROCESS OF SUBJECTING WOOD AND SIMILAR MATERIALS TO A PRELIMINARY TREATMENT FOR THE MANUFACTURE OF PAPER, BOARD, ETC.

No Drawing. Application filed May 29, 1925, Serial No. 33,841, and in Czechoslovakia May 30, 1924.

This invention relates to the process of subjecting wood and similar materials to a preliminary treatment in the manufacture of paper, board, etc. In the known processes applied to this purpose the wood, etc., is steamed for several hours in boilers and, before its removal from these boilers, cooled by various means or, after a short preliminary steaming, boiled in water for the purpose of softening the fibres. The strength of papers produced from wood treated in the manner indicated is not very great while it has been found impossible to dye such papers which usually show a dark color in lighter shades. I am aware that processes are known to boil the wood in vacuum in order to prevent the dark color of the paper and to employ for this purpose the usual chemicals. The application of this process will undoubtedly facilitate dyeing, but the strength of the paper produced thereby remains unsatisfactory while, in addition, this process is, as a rule, very cumbersome and expensive.

The present invention eliminates these drawbacks by dividing the steaming or boiling process into several successive steps or phases by altering the steam pressure and by subjecting the wood, etc., to a prolonged water treatment with or without the addition of chemicals or with and without pressure.

The steaming or boiling process according to the present invention is, for example, divided into four phases. The first phase operates with increasing steam pressure to a pressure of 2-4 atmospheres above atmosphere whereby a gradual warming of the wood in a boiler of known design is effected. During the second phase the steam pressure remains approximately stationary for about 2-4 hours while a certain amount of drying and a partial gasification of the volatile particles of the wood takes place. This partial gasification continues for a while during the third phase, whereupon the boiler pressure is gradually reduced to atmospheric within 3-8 hours so as to cause par-

tial condensation of the steam in the wood. In the fourth phase water with or without 50 chemical admixtures is supplied, and the wood thoroughly saturated for a period of 4, 5 or more hours with water or with the water and the chemicals added to it.

The wood may be subjected to the first 55 three phases either once or as often as desired, and the phases may be of equal or varying duration while the degree of steam pressure may be adapted to the nature of the material and the purpose for which it is 60 intended.

The order of succession of the first three phases mentioned above may be altered to suit the requirements of certain kinds of wood or prepare it for the manufacture of 65 special kinds of paper, but the fourth and final phase of the process always consists in thoroughly saturating the wood with water which may or may not contain chemicals.

I claim:

The process of subjecting wood and similar materials to a preliminary treatment in the manufacture of paper, board or equivalent products consisting in dividing the steaming process into four successive 75 and separate steps, the first step comprising a slow preparatory heating of the material to be treated up to a pressure of 2-4 atmospheres above atmospheric, according to the 80 quality to be produced, while, during the second step, this pressure is kept approximately constant for about 2-4 hours and, during the third step, gradually reduced to atmospheric within 3-8 hours by regulating the steam supply; the fourth step consisting 85 in the admission of water to the boiler, with or without an admixture of chemicals, for the purpose of subjecting the material to constant saturation for a period of 4, 5 or more hours, while the first three steps can 90 be repeated once or several times before such saturation takes place.

In testimony whereof I have affixed my signature.

HUBERT BRÄUNLICH,